

June 23, 1953

H. W. PORTH

2,642,764

METHOD OF ROLLING THIN SHEET METAL

Filed March 15, 1946



INVENTOR  
*Henry W. Porth*  
BY  
Tesch and Darbo  
Atty.



Rolls 15 and 16 are driven and are heated to a temperature of 200° to 300° F. by means which are not shown. The rolled strip then passes through the exit heater 17, around freely rotating guide rolls 18 and 19 and is then wound into a coil upon the reel 20. The exit heater serves to anneal the rolled strip and facilitates the leveling of irregularities under the influence of the tension exerted by reel 20. It also assists, by heat conduction through the strip, in maintaining the portion between the rolls at a satisfactory rolling temperature. Reel 20 is driven, by means which are not shown, at such a rate as to maintain the portion of the strip between it and the reducing rolls 15 and 16 under a definite constant tension such that irregularities in the strip are leveled and the direction of motion of the strip is constant and the edges of the layers in the final coil are even.

As is shown in the drawing, the exit end of the heater 14 is arranged so that it is in close proximity to the point where the strip 10 passes into contact with the reducing rolls 15 and 16. To accomplish this, said exit end portion is tapered, the tapered portion approaching closely to the surfaces of the rolls as they approach each other for the rolling of the strip. The purpose is to reduce to a minimum the time which elapses between the emergence of the strip 10 from the heater 14 and its passage between the rolls 15 and 16. The entrance end of the exit heater 17 is preferably also tapered and arranged to approach the reducing rolls as closely as possible.

The arrangement is such that the temperature of the strip 10 when it is between the reducing rolls, is between approximately 435° F. and 600° F. This is the range of temperature which is suitable for rolling, i. e., within which the material readily undergoes plastic flow and is not injuriously affected. There is a drop in temperature as the strip passes between the reducing rolls. The latter are at a temperature of 200° F. to 300° F., as described heretofore, which is lower than the temperature of the strip, and heat is transferred to the rolls by conduction. There may also be a drop in temperature by radiation during the interval from the time a portion of the strip leaves the heater 14 to the time it makes contact with the reducing rolls. The strip is, therefore, heated to a temperature somewhat above 435° F. in the entrance heater, preferably to a temperature between 500° F. and 600° F. Also, the arrangement is such that the interval from the time a portion of the strip leaves the heater 14 to the time it makes contact with the reducing rolls is short, i. e., preferably not more than one-half of a second, regardless of the speed of travel of the strip. Under such conditions, the strip is sufficiently hot that it readily undergoes plastic flow between the rolls and all of the difficulties mentioned heretofore are avoided. The temperature to which the strip should be heated, within the range of 500° F. to 600° F., depends on the length of time which elapses while the strip passes from the heater 14 to the rolls 15 and 16.

The arrangement is also such that the strip is heated for only a relatively short period of time. This is controlled by regulating the temperature of the heater 14 and the speed of travel of the strip. While the time factor may vary, depending upon the final temperature to which the strip is heated within heater 14, the arrangement is such that a portion of the strip is

at the temperature of 435° F. to 600° F. for not more than three seconds prior to making contact with the reducing rolls. Restricting the interval during which the sheet is at a high temperature serves to restrict the grain growth in the metal and the consequent weakening of the strip.

The exit heater 17 is maintained at a temperature such that the rolled strip is heated at a temperature of approximately 435° F. to approximately 600° F. for a time sufficient to permit annealing and a leveling of the irregularities but insufficient to result in an undesirable grain growth or weakening of the strip. While the time factor may vary, depending upon the temperature to which the strip is heated, the total time during which a portion of the strip is at the temperature of 435° F. to 600° F., that is, the time from the moment it reaches such temperature in entrance heater 14 to the moment it drops below such temperature in or after leaving exit heater 17, should not exceed five seconds. It is preferred that the interval from the time a portion of the strip leaves the reducing rolls until it reaches the exit heater does not exceed one half of a second.

It has been found that with the improved technique described, magnesium sheet material having a thickness of as little as .002 inch can be successfully produced, and the method is useful for sheet material from this thickness up to approximately .01 inch in thickness. With thicknesses greater than .01 inch, the especial procedure of this invention may be convenient but is not essential since the ordinary conventional procedure is satisfactory.

If it is desired that the sheet pass directly from reducing rolls 15 and 16 to a second pair of reducing rolls, such second pair of reducing rolls may be arranged at the exit end of exit heater 17. This may be followed by a third set of reducing rolls with an intervening heater, and so forth until the sheet has been reduced to the desired final thickness. In each heating operation prior to a rolling operation, the strip is heated at a temperature of 500° F. to 600° F. for a period not exceeding three seconds.

While a single embodiment of apparatus suitable for carrying out the invention has been described, this is illustrative only and other apparatus may be used as well. For example, electric current may be passed through the strip material during its travel to the reducing rolls to heat it to the proper temperature, and also as it passes from the reducing rolls to anneal the rolled strip. Apparatus for the electrical heating of strip material either inductively or by contact while it is being rolled are well known and such apparatus may be used in carrying out the present invention.

What is claimed is:

1. In reducing the thickness of sheet material from the group consisting of magnesium and magnesium-base alloys having a thickness of not more than approximately .01 inch by passing said material between reducing rolls, the method which comprises heating said sheet material at a temperature of from approximately 435° F. to approximately 600° F. and maintaining said sheet material at said temperature for a period of time not exceeding approximately 5 seconds during which time said passage between said reducing rolls occurs.

2. The method as claimed in claim 1 in which the heating during passage to the rolls con-

tinues until a time not more than approximately one-half second prior to the time the sheet material reaches the rolls.

3. In the method of reducing the thickness of sheet material from the group consisting of magnesium and magnesium-base alloys having a thickness not exceeding approximately .01 inch by means of pressure rolls, the step which comprises heating said sheet material at a temperature of from approximately 500° F. to approximately 600° F. for a period of time not more than three seconds prior to the time said sheet material reaches said rolls.

4. In reducing the thickness of sheet material from the group consisting of magnesium and magnesium-base alloys having a thickness not exceeding approximately .01 inch by means of pressure reducing rolls, the method which comprises heating said sheet material at a temperature from approximately 500° F. to approximately 600° F. for an interval not exceeding approximately 3 seconds and continuing until a time not more than approximately one-half second prior to the time said sheet material reaches said reducing rolls.

5. In reducing the thickness of sheet material from the group consisting of magnesium and magnesium-base alloys having a thickness not exceeding approximately .01 inch by means of

reducing rolls, the method which comprises heating said sheet material while it is passing both to and from said rolls at a temperature of approximately 435° F. to approximately 600° F. for a total period not exceeding approximately 5 seconds, said heating during passage to said rolls continuing until a time not more than one-half second prior to contact with said rolls and said heating during passage from said rolls starting not more than one-half second subsequent to contact with said rolls.

HENRY W. PORTH.

References Cited in the file of this patent

UNITED STATES PATENTS

| Number    | Name        | Date           |
|-----------|-------------|----------------|
| 1,374,968 | Veazey      | Apr. 19, 1921  |
| 1,480,870 | Thomas      | Jan. 15, 1924  |
| 1,926,057 | Nock et al. | Sept. 12, 1933 |
| 2,149,436 | Hadenfeldt  | Mar. 7, 1939   |

OTHER REFERENCES

The Technology of Magnesium and Its Alloys—  
A translation from the German Magnesium und  
seine Legierungen, compiled by Dr. Ing E. h.  
Adolph Beck. F. A. Hughes and Co., Ltd., 1940,  
pages 387 to 403.